

Feb. 16, 1937.

M. BERGSTEIN

2,071,104

DRY ELECTROLYTIC CONDENSER

Filed May 18, 1931

*Fig. 1.*



*Fig. 2.*



INVENTOR  
Milton Bergstein  
BY  
Frank Crosby & Neal  
ATTORNEY

## UNITED STATES PATENT OFFICE

2,071,104

## DRY ELECTROLYTIC CONDENSER

Milton Bergstein, New York, N. Y., assignor to  
 Micamoid Radio Corporation, Brooklyn, N. Y.,  
 a corporation of New York

Application May 18, 1931, Serial No. 538,401

7 Claims. (Cl. 175—315)

In my copending application, Serial Number 538,399, filed May 18, 1931, entitled "Electrolytic condenser" I have described and claimed electrolytic condensers wherein soaps or mixtures of soaps and fatty acids were employed as constituents of the electrolyte in condensers of the dry electrolytic type, ammonium soaps being preferred on account of the lower solvent action of the ammonium ion on the aluminum oxide film of the condenser.

I have further discovered that the acitivity of the ammonium ion in electrolytes of the above character can be modified by the substitution for the hydrogen atoms of suitable alkyls or alkyl derivatives. For example, the methyl and ethyl ammonium ions are more alkaline, and methanol or ethanol derivatives less alkaline than the unsubstituted ions.

As typical of the compounds capable of giving the effects desired, reference is made to the triethanol ammonium compounds which have the advantage of ready commercial availability, although other alcohol substituted ammonium compounds may be employed.

Triethanol ammonium soaps such as stearate, palmitate or mixtures thereof are quite satisfactory for electrolytic purposes, their consistency being suitable when in solid form and because they can be heated to the melting point without loss of triethanolamine and consequent rapid change in composition, a somewhat objectionable feature in ammonium soaps. Furthermore, their ready fluidity when in liquid form makes it easy to apply them to gauze or other suitable separating medium employed between the armatures of the condenser.

I have found that an electrolyte consisting of triethanol ammonium stearate can be employed without the addition of any other substances whatsoever as the electrolytic conductor in condensers of the above type, it being merely necessary to melt the electrolyte and apply it to a suitable separator medium as known in the art.

I have further found that the addition of triethanol ammonium linoleate lends further desirable properties; for example, the resistance of the electrolyte may be thereby reduced and the effective capacity increased. A mixture in the ratio of two parts by weight of stearate to one part of linoleate, for example, is satisfactory. The unmixed stearate, however, has the advantage of greater solidity, and the necessary period of aging of the condenser is also somewhat increased by the addition of ammonium linoleate, although not to such an extent

as to render the use of the latter impractical.

Ordinary commercial grades of triethanol ammonium soaps are satisfactory for the above purpose, high purity being unnecessary, and electrolytes of the above nature have the advantage of lower cost and more easy application as compared to gum arabic, glycol, glycerol, glucose borate mixtures and the like which are commonly employed.

I may modify the electrolytes of the types above described by the addition of a small quantity, for example, 5% by weight of a weak organic acid such as stearic acid, thereby decreasing the aging period of the condenser and obtaining somewhat higher conductivity in the electrolyte and consequent higher effective capacity; or an equivalent quantity of acid salt of acids of the above type may be added for similar purposes, such as ammonium or aluminum acetate. I find that a convenient way for preparing the aluminum acetate is by the addition of one part of glacial acetic acid to about one and one-half parts by weight of aluminum oxide, yielding a mixture of aluminum acetate, aluminum hydroxide and aluminum oxide. The excess of aluminum oxide furnishes aluminum ion within the electrolyte, thus cutting down the solvent effect of the electrolyte upon the aluminum oxide coat of the electrolyte.

A preferred form of condenser employing the electrolyte above described is shown in the accompanying drawing wherein Fig. 1 is a perspective view of the condenser partially unrolled, and Fig. 2 is an enlarged cross-sectional view taken through the condenser along the line 2—2 of Fig. 1.

In the drawing, the numeral 1 designates one electrode with its terminal 2. The other electrode is designated by 3 with its terminal shown at 4. Between the electrodes are layers of 40 gauze 5 and 6 impregnated with the electrolyte.

I claim:

1. An electrolytic condenser of the class described having an armature of the film-forming type, and an electrolyte consisting of a triethanol ammonium soap.

2. An electrolytic condenser of the class described having an armature of the film-forming type, and an electrolyte consisting of a mixture of triethanol ammonium soaps.

3. An electrolytic condenser of the class described having an armature of the film-forming type, and an electrolyte consisting of a mixture of triethanol ammonium stearate and triethanol ammonium linoleate.

5

10

15

20

25

30

35

40

45

50

55

4. An electrolytic condenser of the class described having an armature of the film-forming type, and an electrolyte consisting of a soap having a substituted ammonium ion and the ion of a soap-forming acid.
5. An electrolytic condenser of the class described having an armature of the film-forming type and an electrolyte consisting of a soap hav-

ing an alcohol substituted ammonium ion and the ion of a weak organic acid.

6. An electrolyte consisting of a soap produced by the reaction of a soap-forming acid and an alcohol substituted amine.

7. An electrolyte consisting of an ethanol ammonium soap.

MILTON BERGSTEIN.